# EUROPEAN PATENT SPECIFICATION

(11) **EP 3 722 467 B1**
(45) Date of publication and mention of the grant of the patent: **10.05.2023**
(21) Application number: 19734225.6
(22) Date of filing: 01.04.2019
(51) Int. Cl.: D02G 3/44, D02G 3/04, D02G 3/38, D04B 1/14, D04B 1/18, D04B 1/28

(54) **METHOD FOR PREPARING TUNGSTEN WIRE TWIST-WRAPPED ANTI-CUT YARN AND METHOD FOR MAKING TEXTILE USING SAME**
VERFAHREN ZUR HERSTELLUNG VON VERZWIRNTEM UND UMWICKELTEM SCHNITTFESTEM GARN AUF WOLFRAMBASIS UND VERFAHREN ZUR HERSTELLUNG VON TEXTILIEN DAMIT
PROCÉDÉ DE PRÉPARATION D'UN FIL ANTI-COUPE ENVELOPPÉ PAR TORSION DE FIL DE TUNGSTÈNE ET PROCÉDÉ DE FABRICATION DE TEXTILE L'UTILISANT

(30) Priority: 20.02.2019 CN 201910125947
(43) Date of publication of application: 14.10.2020
(73) Proprietor: Honghan Nantong Protection of Science & Technology Co., Ltd., Nantong City, Jiangsu 226400 (CN)
(72) Inventor: LIN, Xin, Nantong City, Jiangsu 226400 (CN)
(74) Representative: ZHAOffice SPRL
(86) International application number: PCT/CN2019/080735
(87) International publication number: WO 2020/168616

(56) References cited:
- WO-A1-2018/230945
- CN-A- 1 886 539
- CN-A- 106 087 171
- CN-A- 106 087 171
- CN-A- 106 544 769
- CN-A- 107 541 830
- CN-A- 107 541 830
- CN-A- 108 505 174
- CN-A- 108 505 174
- CN-A- 108 505 200
- RU-C1- 2 075 957
- US-A1- 2018 135 211
- Superiorglove Superiorglove ET AL: "Dyneema Vs. Kevlar : The Ultimate Showdown", , 11 March 2018 (2018-03-11), XP055690022, Retrieved from the Internet: URL:https://web.archive.org/web/2018031107 2711/https://www.superiorglove.com/blog/dy neema-vs-kevlar [retrieved on 2020-04-28]

## Description

### Technical Field

The present invention relates to the field of yarns, and in particular, to a method of producing tungsten twist-coated and wrapped cut-resistant yarn, and a method of producing a textile using same.

### Background

Cut-resistant gloves are functional gloves. To achieve cut resistance, the thickness of current cut-resistant gloves is usually increased. The increase in thickness enhances the cut resistance of the gloves, but brings an uncomfortable feeling to a user. The gloves are stiff, thick and heavy, and do not bend easily, increasing the burden on an operator.

In prior art documents various cut-resistant materials have been discussed and described:
Russian patent RU 2 075 957 describes a haberdashery product for protection against cuts in a glove, at least the working part of which consists of a shell connected to a fabric lining and having an elastomeric coating on the outer surface. The glove comprises a yarn comprising a core made with a metal wire, the core itself comprises a metal wire with a diameter of 0.06-0.09 mm twisted with a further synthetic thread, around the core two layers of twisting synthetic thread are provided, a twisting synthetic thread of one of the layers around the core is made on the basis of polyamidobenzimidazole terephthalamide or copolyparaphenylene terephthalamide, and the synthetic thread of the other layer is made of polyester or polyamide thread. Chinese patent application CN 1085 05 174 discloses tungsten filament blending cutting resistance yarns and a preparation method thereof, a glove body and a spinning product. The preparation method for the tungsten filament blending cutting resistance yarn comprises the following steps (1): tungsten filaments are taken as core yarns, and two layers of polyester filaments are wrapped around the core yarns, to make a double polyester covered tungsten yarn, next to this double polyester covered tungsten yarn a spandex yarn is provided; around this double core yarn polyamide yarns are wrapped and finally ultra high molecular weight polyethylene fibers are wrapped around the whole.

The article "Dyneema Vs. Kevlar: the ultimate showdown" dated 11 March 2018 by Superior Glove compares in some general terms the properties of Dyneema and Kevlar in gloves.

The Chinese patent application CN 106 087 171 discloses a novel cut-resistant yarn and production method of cut-resistant articles of the novel cut-resistance yarn; the novel cut-resistant yarn is woven by: using a high-strength high-count tungsten filament yarn as a core yarn, covering the core yarn with wrapping fiber/yarn, and spinning.

The United States patent application US2018/135211 discloses a hybrid fiber which includes: a metal wire having a roughened surface. In the hybrid fiber, the metal wire and the fiber are combined.

The Chinese patent application CN 107 541 830 discloses a tungsten-core yarn and a yarn forming process and also relates to a protective textile produced by using the yarn and a knitting method of the protective textile.

### Summary of the Invention

To solve the foregoing technical problem, the present invention provides a method of producing a tungsten twist-coated and wrapped cut-resistant yarn, and a method of producing a textile using same.

The present invention adopts the following technical solution:
A method of producing a tungsten twist-coated and wrapped cut-resistant yarn includes the following operation steps:
a. obtaining tungsten filament twist-coated yarn: twisting together an auxiliary yarn I and one or more of tungsten filaments at a twist of 400 to 700 twists/meter, the auxiliary yarn I being made from one of nylon, polyester, cotton, bamboo fiber, and tencel and having a linear density of 40 D to 140D (4,44 Tex to 15,55 Tex) and the one or more of tungsten filaments having diameters of 0.02 mm, 0.025 mm, or 0.03 mm and
b. producing the tungsten twist-coated and wrapped cut-resistant yarn: wrapping a high-molecular-weight polyethylene yarn around the tungsten filament twist-coated yarn obtained in step a, at a twist of 120 to 280 twists/meter, wherein the polyethylene fiber has a molecular weight of 10MW to 500MW and a linear density of 50D to 400D (5,55 Tex to 44,44 Tex).

Further, in the tungsten filament twisted yarn in step a, preferably the tungsten filament accounts for 35% to 75%, and the auxiliary yarn I accounts for 25% to 65%.

Further, preferably the auxiliary yarn I is made from nylon and the linear density of the nylon is preferably 40D, 50D, 70D, 100D or 140D (4,44 Tex, 5,55 Tex, 7,77 Tex, 11,11 Tex or 15,55 Tex).

Further, preferably in the tungsten twist-coated and wrapped cut-resistant yarn in step b, the tungsten filament twist-coated yarn accounts for 35% to 65%, and the polyethylene fiber accounts for 35% to 65%.

Further, preferably the linear density of the polyethylene yarn is preferably 50D, 100D, 150D, 200D, 300D, or 400D (5,55 Tex, 11,11 Tex, 16,66 Tex, 22,22 Tex, 33,33 Tex or 44,44 Tex). A method of producing a textile from tungsten twist-coated and wrapped cut-resistant yarn produced according to any of the claims 1 to 5 includes: by a knitting process with double yarn feeders, producing a textile from spandex stretch yarn and the tungsten twist-coated and wrapped cut-resistant yarn produced according to any of the claims 1 to 5, wherein the tungsten twist-coated and wrapped cut-resistant yarn accounts for 60% to 80%, and the spandex stretch yarn accounts for 20% to 40% and the spandex stretch yarn is made from nylon-wrapped spandex, polyester-wrapped spandex, or polyethylene-fiber-wrapped spandex; and is made by twisting together a spandex filament with a linear density of 20D to 100D (2,22 Tex to 11,11 Tex) and auxiliary yarn II with a linear density of 50D to 200D (5,55 Tex to 22,22 Tex) at the twist of 180 to 580 twists/meter, wherein the auxiliary yarn II is made from nylon, polyester or polyethylene; and the tension ratio of the spandex stretch yarn preferably ranges from 1.5 to 2.4.

The present invention achieves the following advantageous effects: 1. A tungsten filament with rigidity of 9, ranking only second to diamond, is used as the raw material. Therefore, textiles produced with this material are highly rigid, thin and light. Moreover, China is a major producer of tungsten filaments, and the reserves account for 75% of the world's total reserves. Therefore, the present invention has advantages of a broad variety of raw material sources and low costs. 2. The produced textiles are light, thin, and soft; and have high cut resistance, chemical stability, bending resistance, and deformation resistance during washing, and excellent electrical conductivity. Further, the textiles can reach a cut resistance grade of A6 or higher in the ASTM standard; an ISO grade of F or higher in the European standard; and a wear resistance grade of 4, cut resistance grade of 5, tear resistance grade of 4, and puncture resistance grade of 4 in the European Union (EN) 388 standard.

### Brief Description of the Drawings

FIG. 1 is a schematic structural diagram of tungsten filament twist-coated yarn in the present invention (using one strand of auxiliary yarn I and one tungsten filament);
FIG. 2 is a schematic structural diagram of tungsten filament twist-coated yarn in the present invention (using one strand of auxiliary yarn I and two or more tungsten filaments);
FIG. 3 is a schematic structural diagram of tungsten twist-coated and wrapped cut-resistant yarn in the present invention (using one strand of auxiliary yarn I, one tungsten filament, and one polyethylene yarn);
FIG. 4 is a schematic structural diagram of tungsten twist-coated and wrapped cut-resistant yarn in the present invention (using one strand of auxiliary yarn I, two or more tungsten filaments, and one polyethylene yarn); and
FIG. 5 is a schematic structural diagram of spandex stretch yarn in the present invention.

Meanings of numerals in the drawings:
1. Auxiliary yarn I, 2. Tungsten filament, 3. Polyethylene yarn,
4. Spandex filament, and
5. Auxiliary yarn II

### Detailed Description

In order to further understand the present invention, the present invention is further described in detail below with reference to examples and the accompanying drawings. The examples are only intended to explain the present invention, and not to limit the protection scope of the present invention.

A method of producing tungsten twist-coated and wrapped cut-resistant yarn includes the following operation steps:
a. obtaining of tungsten filament twist-coated yarn: As shown in FIG. 1 and FIG. 2, auxiliary yarn I 1 and a tungsten filament 2 are twisted at a twist of 400 to 700 twists/meter, to obtain the tungsten filament twist-coated yarn. The tungsten filament preferably accounts for 35% to 75%, and the auxiliary yarn I 1 accounts for 25% to 65%. The auxiliary yarn I 1 is made from one of nylon, polyester, cotton, bamboo fiber, and tencel; and has a linear density of 40D to 140D (4,44 Tex to 15,55 Tex).
   The tungsten filament 2 is selected to be one tungsten filament having a diameter of 0.02 mm, 0.025 mm, or 0.03 mm.
b. Production of tungsten twist-coated and wrapped cut-resistant yarn: As shown in FIG. 3 and FIG. 4, a high-molecular-weight polyethylene fiber 3 is wrapped around the tungsten filament twist-coated yarn obtained in step a, at a twist of 120 to 280 twists/meter, to produce the tungsten twist-coated and wrapped cut-resistant yarn. In the tungsten twist-coated and wrapped cut-resistant yarn, the tungsten twist-coated yarn preferably accounts for 35% to 65%, and the polyethylene fiber 3 accounts for 35% to 65%. The polyethylene yarn has a molecular weight of 10MW to 500MW and a linear density of 50D to 400D (5,55 Tex to 44,44 Tex). The linear density of the polyethylene yarn is preferably 50D, 100D, 150D, 200D, 300D, or 400D (5,55 Tex, 11,11 Tex, 16,66 Tex, 22,22 Tex, 33,33 Tex or 44,44 Tex).

Afterwards, a method of producing a textile using the tungsten twist-coated and wrapped cut-resistant yarn as described above is as follows: By a knitting process with double yarn feeders, a textile is produced from spandex stretch yarn and the tungsten twist-coated and wrapped cut-resistant yarn. The tungsten twist-coated and wrapped cut-resistant yarn accounts for 60% to 80%, and the spandex stretch yarn accounts for 20% to 40%. The spandex stretch yarn is made from nylon-wrapped spandex, polyester-wrapped spandex, or polyethylene-fiber-wrapped spandex. As shown in FIG. 5, the spandex stretch yarn is made by twisting together a spandex filament 4 with a linear density of 20D to 100D (2,22 Tex to 11,11 Tex) and auxiliary yarn II 5 with a linear density of 50D to 200D (5,55 Tex to 22,22 Tex) at the twist of 180 to 580 twists/meter. The auxiliary yarn II is made from nylon, polyester or polyethylene; and the tension ratio of the spandex stretch yarn preferably ranges from 1.5 to 2.4.

Data and detection results, regarding textiles produced by the method of producing tungsten twist-coated and wrapped cut-resistant yarn and by the method of producing a textile using the yarn, in five comparative examples and eleven examples are shown below:

| Sample No. | Diameter of the tungsten filament (mm) | Fineness of the auxiliary yarn I (D) | Fineness of the polyethylene fiber (D) | Fineness of the spandex filament (D) | Fineness of the auxiliary yarn II (D) | Weight (g/piece) | Cut resistance (ASTM) |
|---|---|---|---|---|---|---|---|
| comparative example 1 | 0.006 | 70 | 50 | 20 | 100 | 13.5 | A4 |
| comparative example 2 | 0.01 | 30 | 100 | 30 | 200 | 14.5 | A4 |
| comparative example 3 | 0.015 | 70 | 100 | 140 | 100 | 15 | A4 |
| comparative example 4 | 0.015 | 100 | 150 | 40 | 250 | 15.5 | A5 |
| comparative example 5 | 0.015 | 100 | 200 | 70 | 250 | 16 | A5 |
| Example 1 | 0.02 | 50 | 100 | 20 | 70 | 16.8 | A6 |
| Example 2 | 0.02 | 70 | 150 | 40 | 100 | 17 | A6 |
| Example 3 | 0.02 | 100 | 200 | 30 | 70 | 17.8 | A7 |
| Example 4 | 0.02 | 70 | 200 | 20 | 140 | 18.8 | A7 |
| Example 5 | 0.025 | 70 | 150 | 30 | 100 | 18 | A6 |
| Example 6 | 0.025 | 100 | 200 | 40 | 70 | 19 | A6 |
| Example 7 | 0.025 | 140 | 200 | 70 | 100 | 19 | A7 |
| Example 8 | 0.03 | 140 | 200 | 40 | 140 | 19 | A6 |
| Example 9 | 0.03 | 70 | 200 | 40 | 70 | 19.2 | A6 |
| Example 10 | 0.03 | 100 | 300 | 70 | 140 | 20 | A7 |
| Example 11 | 0.03 | 100 | 300 | 100 | 100 | 20 | A8 |

| | | | | | | | |
|---|---|---|---|---|---|---|---|
| Note: The auxiliary yarn I in the comparative examples 1 to 3 and the examples 1 to 4 is made from nylon; the auxiliary yarn I in the comparative examples 4 and 5 and the examples 5 to 8 is made from polyester; the auxiliary yarn I in the examples 9 to 11 is made from cotton; the auxiliary yarn II in the comparative examples 1 to 3 and the examples 1 to 4 is made from nylon; the auxiliary yarn II in the comparative examples 4 and 5 and the examples 5 to 8 is made from polyester; and the auxiliary yarn II in the examples 9 to 11 is made from polyethylene. | | | | | | | |

It can be seen from the above examples and comparative examples that, the textiles produced within the data ranges of the present claims can all reach a cut resistance grade of A6 or higher in the ASTM standard.

## Claims

1. A method of producing a tungsten twist-coated and wrapped cut-resistant yarn, comprising the following operation steps:
a. producing a tungsten filament twist-coated yarn: an auxiliary yarn I (1) and one or more tungsten filaments (2) are twisted with a twist of 400 to 700 twists/meter, wherein the auxiliary yarn I (1) is made from one of nylon, polyester, cotton, bamboo fiber, and tencel and has a linear density of 40D to 140D (4,44 Tex to 15,55 Tex) and the one or more of tungsten filaments having diameters of 0.02 mm, 0.025 mm, or 0.03 mm; and
b. producing the tungsten twist-coated and wrapped cut-resistant yarn: wrapping a high-molecular-weight polyethylene yarn (3) around the tungsten filament twist-coated yarn obtained in step a, at the twist of 120 to 280 twists/meter wherein the high-molecular-weight polyethylene yarn (3) has a molecular weight of 10MW to 500MW and a linear density of 50D to 400D (5,55 Tex to 44,44 Tex).

2. The method of producing a tungsten twist-coated and wrapped cut-resistant yarn according to claim 1, wherein in the tungsten filament twist-coated yarn in step a, the tungsten filament (2) accounts for 35% to 75%, and the auxiliary yarn I (1) accounts for 25% to 65%.

3. The method of producing a tungsten twist-coated and wrapped cut-resistant yarn according to claim 1, wherein the auxiliary yarn I (1) is made from nylon and the linear density of the nylon is 40D, 50D, 70D, 100D, or 140D (4,44 Tex, 5,55 Tex, 7,77 Tex, 11,11 Tex or 15,55 Tex).

4. The method of producing a tungsten twist-coated and wrapped cut-resistant yarn according to any of preceding claims , wherein in the tungsten twist-coated and wrapped cut-resistant yarn in step b, the tungsten filament twist-coated yarn accounts for 35% to 65%, and the polyethylene yarn (3) accounts for 35% to 65%.

5. The method of producing tungsten twist-coated and wrapped cut-resistant yarn according to claim 1, wherein the linear density of the polyethylene yarn (3) is 50D, 100D, 150D, 200D, 300D, or 400D (5,55 Tex, 11,11 Tex, 16,66 Tex, 22,22 Tex, 33,33 Tex or 44,44 Tex).

6. A method of producing a textile from tungsten twist-coated and wrapped cut-resistant yarn produced according to any of the claims 1 to 5, comprising: by a knitting process with double yarn feeders, producing a textile from a spandex stretch yarn (4) and the tungsten twist-coated and wrapped cut-resistant yarn produced according to any of the claims 1 to 5, wherein the tungsten twist-coated and wrapped cut-resistant yarn accounts for 60% to 80%, and the spandex stretch yarn accounts for 20% to 40% and the spandex stretch yarn is made from nylon-wrapped spandex, polyester-wrapped spandex, or polyethylene-fiber-wrapped spandex; and is made by twisting together a spandex filament with a linear density of 20D to 100D (2,22 Tex to 11,11 Tex) and an auxiliary yarn II (5) with a linear density of 50D to 200D (5,55 Tex to 22,22 Tex) at the twist of 180 to 580 twists/meter, the auxiliary yarn II being made from nylon, polyester or polyethylene.

7. A method of producing a textile from tungsten twist-coated and wrapped cut-resistant yarn according to claim 6, wherein the tension ratio of the spandex stretch yarn ranges from 1.5 to 2.4.

## Patentansprüche

1. Verfahren zur Herstellung eines zwirnbeschichteten und umwickelten schnittfesten Garns auf Wolframbasis, die folgenden Schritte umfassend:
a. Herstellung eines zwirnbeschichteten Garns auf der Basis von Wolframfilamenten: ein Hilfsgarn I (1) und ein oder mehrere Wolframfilamente (2) werden mit einem Zwirn von 400 bis 700 Zwirnen/Meter verzwirnt, wobei das Hilfsgarn I (1) aus einem Material ausgewählt aus Nylon, Polyester, Baumwolle, Bambufaser und Tencel hergestellt wird und eine lineare Dichte von 40 D bis 140 D (4.44 Tex bis 15,55 Tex ) aufweist, und die ein oder mehrere Wolframfilamente Durchmesser von 0,02 mm, 0,025 mm oder 0,03 mm aufweisen; und
b. Herstellung des zwirnbeschichteten und umwickelten schnittfesten Garns auf Wolframbasis: Umwicklung eines Garns aus hochmolekularem Polyethylen (3) um das zwirnbeschichtete Garn auf der Basis von Wolframfilamenten im Schritt a erhalten, mit einem Zwirn von 120 bis 280 Zwirnen/Meter, wobei das hochmolekulare Polyethylen (3) ein Molekulargewicht von 10 MW bis 500 MW und eine lineare Dichte von 50 D bis 400 D (5,55 Tex bis 44,44 Tex) aufweist.

2. Verfahren zur Herstellung eines zwirnbeschichteten und umwickelten schnittfesten Garns auf Wolframbasis nach Anspruch 1, wobei in dem zwirnbeschichteten Garn auf der Basis von Wolframfilamenten des Schritts a, das Wolframfilament (2) 35 % bis 75 % beträgt, und das Hilfsgarn I (1) 25% bis 65% beträgt.

3. Verfahren zur Herstellung eines zwirnbeschichteten und umwickelten schnittfesten Garns auf Wolframbasis nach Anspruch 1, wobei das Hilfsgarn I (1) aus Nylon ist, und die lineare Dichte des Nylons 40 D, 50 D, 70 D, 100 D oder 140 D (4,44 Tex, 5,55 Tex, 7,77 Tex, 11,11 Tex oder 15,55 Tex) ist.

4. Verfahren zur Herstellung eines zwirnbeschichteten und umwickelten schnittfesten Garns auf Wolframbasis nach einem der vorhergehenden Ansprüche, wobei in dem zwirnbeschichteten und umwickelten schnittfesten Garn auf Wolframbasis des Schritts b, das zwirnbeschichtete Garn auf der Basis von Wolframfilamenten 35 % bis 65 % beträgt, und das Polyethylengarn (3) 35% bis 65% beträgt.

5. Verfahren zur Herstellung eines zwirnbeschichteten und umwickelten schnittfesten Garns auf Wolframbasis nach Anspruch 1, wobei die lineare Dichte des Polyethylengarns 50 D, 100 D, 150 D, 200 D, 300 D, oder 400 D (5,55 Tex, 11,11 Tex, 16,66 Tex, 22,22 Tex, 33,33 Tex oder 44,44 Tex) ist.

6. Verfahren zur Herstellung von Textilien aus einem zwirnbeschichteten und umwickelten schnittfesten Garn auf Wolframbasis nach einem der Ansprüche 1 bis 5, umfassend: durch ein Strickverfahren mittels einer doppelten Garnzuführung, Herstellung von Textilien aus einem dehnbaren Elastangarn (4) und dem zwirnbeschichteten und umwickelten schnittfesten Garns auf Wolframbasis nach einem der Ansprüche 1 bis 5 hergestellt, wobei das zwirnbeschichtete und umwickelte schnittfeste Garn auf Wolframbasis 60% bis 80 % beträgt, und das dehnbare Elastangarn 20 % bis 40 % beträgt, und das dehnbaren Elastangarn aus mit Nylon umwickeltem Elastan, mit Polyester umwickeltem Elastan, oder mit Polyethylen umwickeltem Elastan hergestellt wird; und durch gleichzeitiges Verzwirnen eines Elastans mit einer linearen Dichte von 20 D bis 100 D (2,22 Tex bis 11,11 Tex) und eines Hilfsgarns II (5) mit einer linearen Dichte von 50D bis 200 D (5,55 Tex bis 22,22 Tex) bei dem Zwirn von 180 bis 580 Zwirnen/Meter hergestellt wird, wobei das Hilfsgarn II aus Nylon, Polyester oder Polyethylene hergestellt wird.

7. Verfahren zur Herstellung eines zwirnbeschichteten und umwickelten schnittfesten Garns auf Wolframbasis nach Anspruch 6, wobei das Spannungsverhältnis des dehnbaren Elastangarn von 1,5 bis 2,4 variiert.

## Revendications

1. Procédé de production de fil résistant à la coupure enveloppé et revêtu par torsion à base de tungstène, comprenant les étapes suivantes :
a. production d'un fil revêtu par torsion à filament de tungstène : un fil auxiliaire I (1) et un ou plusieurs filaments de tungstène (2) sont torsadés avec une torsion de 400 à 700 torsions par mètre, où le fil auxiliaire I (1) est fabriqué à partir d'une matière parmi un nylon, un polyester, de la fibre de bambou, du coton et du tencel et présente une densité linéaire de 40 D à 140 D (4,44 Tex à 15,55 Tex) et où ledit un ou plusieurs filaments de tungstène présentent des diamètres de 0,02 mm, 0,025 mm ou de 0,03 mm ; et
b. production du fil résistant à la coupure enveloppé et revêtu par torsion à base de tungstène : enroulement d'un fil en polyéthylène à haut poids moléculaire (3) autour du fil revêtu par torsion à filament de tungstène obtenu à l'étape a avec une torsion de 120 à 280 torsions par mètre, où le fil en polyéthylène à haut poids moléculaire (3) présente un poids moléculaire de 10 MW à 500 MW et une densité linéaire de 50 D à 400 D (5.55 Tex à 44,44 Tex).

2. Procédé de production de fil résistant à la coupure enveloppé et revêtu par torsion à base de tungstène selon la revendication 1, dans lequel, dans le cas du fil revêtu par torsion de filament de tungstène de l'étape a, le filament de tungstène (2) compte pour 35 % à 75 % et le fil auxiliaire I (1) compte pour 25 % à 65 %.

3. Procédé de production de fil résistant à la coupure enveloppé et revêtu par torsion à base de tungstène selon la revendication 1, dans lequel le fil auxiliaire I (1) est fabriqué en nylon et la densité linéaire du nylon est de 40 D, 50 D, 70 D, 100 D, ou de 140 D (4,44 Tex, 5,55 Tex, 7,77 Tex, 11,11 Tex ou 15,55 Tex).

4. Procédé de production de fil résistant à la coupure enveloppé et revêtu par torsion à base de tungstène selon l'une quelconque des revendications précédentes, dans lequel, dans le cas du fil revêtu par torsion de filament à base de tungstène de l'étape b, le fil revêtu par torsion à filament de tungstène compte pour 35 % à 65 % et le fil de polyéthylène compte pour 35 % à 65 %.

5. Procédé de production de fil résistant à la coupure enveloppé et revêtu par torsion à base de tungstène selon la revendication 1, dans lequel la densité linéaire du fil de polyéthylène est de 50 D, 100 D, 150 D, 200 D, ou de 400 D (5,55 Tex, 11,11 Tex, 16,66 Tex, 22,22 Tex, 33,33 Tex ou 44,44 Tex).

6. Procédé de production d'un textile à partir de fils résistant à la coupure enveloppés et revêtus par torsion à base de tungstène selon l'une quelconque des revendications 1 à 5, comprenant : par un procédé de tricotage au moyen d'un double dispositif d'alimentation en fil, production d'un textile à partir de fil extensible en élasthanne (4) et de fil résistant à la coupure enveloppé et revêtu par torsion à base de tungstène produit selon l'une quelconque des revendications 1 à 5, où le fil résistant à la coupure enveloppé et revêtu par torsion à base de tungstène compte pour 60 % à 80 %, et le fil extensible en élasthanne compte pour 20% à 40 %, et le fil extensible en élasthanne est fabriqué à partir d'élasthanne enveloppé par du nylon, d'élasthanne enveloppé par du polyester, ou à partir d'élasthanne enveloppé par des fibres de polyéthylène ; et le fil extensible d'élasthanne est fabriqué en torsadant ensemble un filament d'élasthanne présentant une densité linéaire de 20 D à 100 D (2,22 Tex à 11,11 Tex) et un fil auxiliaire II (5) présentant une densité linéaire de 50 D à 200 D (5,55 Tex à 22,22 Tex) pour une torsion de 180 à 580 torsions par mètre, le fil auxiliaire II étant fabriqué à partir de nylon, de polyester ou de polyéthylène.

7. Procédé de production d'un textile à partir de fils résistant à la coupure enveloppés et revêtus par torsion à base de tungstène selon la revendication 6, dans lequel le rapport des tensions dans l'élasthanne varie de 1,5 à 2,4.
